

E. E. NOVOTNY.

PRINTING PLATE.

APPLICATION FILED DEC. 11, 1919

1,377,518.

Patented May 10, 1921.

*Fig. 1.*



*Fig. 2.*



*Fig. 3.*



*Fig. 4.*



*Fig. 5.*



Inventor

Emil E. Novotny  
By his Attorneys  
Meyers, Cushman & Pea

# UNITED STATES PATENT OFFICE.

EMIL E. NOVOTNY, OF LOGAN, PENNSYLVANIA, ASSIGNOR TO JOHN STOGDELL  
STOKES, OF PHILADELPHIA, PENNSYLVANIA.

## PRINTING-PLATE.

1,377,518.

Specification of Letters Patent. Patented May 10, 1921.

Application filed December 11, 1919. Serial No. 344,229.

*To all whom it may concern:*

Be it known that I, EMIL E. Novotny, a citizen of the United States, and a resident of Logan, in the county of Philadelphia and 5 State of Pennsylvania, have invented certain new and useful Improvements in Printing-Plates, of which the following is a specification.

This invention relates to certain novel 10 and useful improvements in printing plates, and has particular application to printing plates which are composed in whole or in part of phenolic condensation products such as bakelite, condensite or the like, or in fact 15 of any other synthetic resin possessing characteristics which render the same suitable for the making of such plates; for instance the capability of hardening and setting to an infusible form during or after the plate 20 molding operation.

As is well known, these phenolic condensation products are capable of reduction by heat to a plastic state, and of subsequently 25 hardening and setting under heat and pressure, or heat, pressure and cooling to a hard permanent state. I have used such material to great advantage in making durable and high grade printing plates, especially where I have made the body of the plate of fiber 30 or fiber board sheets impregnated with the phenolic condensation product.

However it sometimes happens that a plate 35 will be produced which will be found to be buckled or warped so as to practically render it useless for press work. Usually the production of such buckled or warped plates is due to carelessness on the part of the operator 40 in charge of the molding press on which the plates are made. It is very desirable to save these buckled or warped plates and to remedy the defect so that such plates may be used for printing instead of being discarded.

One of the principal objects of the invention therefore is the production of a molded 45 printing plate wherein warping or buckling of the plate will be prevented or, if warping or buckling exists in the plate, such defect may be eliminated.

It is also my purpose to provide a printing plate which will embrace the desired features of simplicity, accuracy and durability, and which may be manufactured and marketed at a relatively low cost.

With the above recited objects and others 55 of a similar nature in view my invention

consists in the improved printing plate and in the method set forth in and falling within the scope of the appended claims:

In the accompanying drawing:

Figure 1, is a view in cross section of a 60 phenolic printing plate which has warped or buckled.

Fig. 2, is a similar view of a backing section or slab which is to be united with the back of the warped plate to eliminate the 65 defect.

Fig. 3, conventionally illustrates the platens of a press and showing the step of applying the backing to the warped plate.

Fig. 4, is a cross sectional view showing 70 the corrected plate.

Fig. 5, is a cross sectional view and illustrating a plate backed up to avoid warping and then mounted upon a wooden base block.

In making a printing plate I may proceed 75 as follows:

I select a sheet of stock of suitable size, and which may be either made entirely of a phenolic condensation product, or of such product in combination with other materials 80 such as fiber.

The preferred way of preparing this stock is to impregnate a sheet of fiber board with a certain amount of phenolic material and then place this impregnated sheet between 85 the flat platens of the press and apply heat and pressure to a degree sufficient to bring some of the phenolic material to the face of the fiber board sheet where it is partially hardened or set so as to provide smooth, polished faces for a sheet, not yet set to such a degree that will prevent the further working of the material in the subsequent making of the plate. To the back face of the sheet of stock I apply a sheet or layer, preferably 95 composed of bond paper or other absorbent material, which has been saturated with a low percentage phenolic solution or varnish, and then heated and dried until the phenolic material therein has assumed an infusible 100 form. The result will be that this paper sheet so treated will retain its rough, stratified characteristics and will be rendered non-absorbent by the phenolic material, so that the fiber structure of the paper will not disintegrate or swell when wet by the cleaning 105 solutions commonly used on presses and printing equipment. This paper-backed sheet is then placed face down on the printing plate matrix in a suitably heated press 110

and the plate is molded against the matrix in the usual way. The molded plate, when completed, may through carelessness on the part of the operator, or because of some peculiarity or deficiency in the material, or for some other reason, appear warped or buckled as indicated; for example in Fig. 1 of the drawing wherein the numeral 1 indicates the phenolic plate proper and 2 is the phenolic treated sheet of paper or the like which has been applied to the back of the plate 1 and which, of course, has been caused to adhere thereto during the molding operation by the phenolic material at the back surface 15 of the plate, this material when soft being exceedingly sticky in its nature, but subsequently, of course, hardening to a set form.

To eliminate the buckling or warping in the plate, as illustrated in Fig. 1, I then 20 proceed as follows:

Upon the top surface of the paper backing 2 of the plate 1, I apply a coating 3 of a suitable cement, preferably water-glass. I then impose upon this cement coated backing 25 2, a backing sheet or layer 4 shown in Fig. 2. This backing sheet 4 is composed preferably of fiber board impregnated with phenolic material and preliminarily molded, as described for the plate blank, to form 30 a slab having flat smooth polished faces. The backing slab 4 and the plate thus assembled are placed in a flat press and subjected to slight pressure, without heating, for a short period of time, say one half 35 minute, until the plate and the back 4 are firmly united. As the plate 1, owing to its inherent structure can yield or spring slightly it will be flattened in the press at the time of the application of the backing 40 slab, and when removed from the press the backing slab will support the plate 1 and maintain the same in a substantially flat condition. The plate will not subsequently 45 warp because the backing slab or sheet has been set to a permanent flat condition and as the plate 1 has been pressed and cemented into a firm union with the backing slab, the latter of course will prevent the subsequent warping of the plate. Should any slight 50 buckling occur it will not interfere with the proper use of the plate on the press as the press hooks will hold the plate securely and properly on the press bed, the plate being relatively thin and capable of slight flexing 55 to press it into place on the bed of the press beneath the hooks. If desired, of course, the coating of water-glass cement might be applied to the contacting face of the backing slab 4 instead of to the absorbent paper 2 60 at the back of the plate 1.

Furthermore, I prefer to apply to the back of the backing slab 4 a sheet of paper, such as bond paper or the like, shown at 5, which has also been treated with phenolic 65 material like the sheet 2. When desired, this

sheet 5 may be coated with the same water-glass solution or cement and the plate with its backing slab then firmly mounted upon a wooden base or block 6, as shown in Fig. 5, the union of the back plate with the base 70 block being completed by subjecting these assembled elements to pressure in a press. This manner of mounting the plate upon a wooden base block is very advantageous, as it dispenses with the necessity of drilling 75 the plate and nailing the same to the wood base. In the electrotyping trade it is possible to fasten plate to wooden base blocks and the like by using a nailing machine whereas these hard, brittle phenolic plates 80 require drilling and hand nailing because of the impracticability of making nails driven by a nailing machine coincide properly with holes previously drilled through the phenolic plate. 85

My herein described method of cementing or gluing the elements together, utilizing the phenolic treated paper sheets, permits the glue or cement to absorb and set rapidly so that the plate is ready for use in a short 90 time. Furthermore, the interposed phenolic treated sheets constitute separating mediums in the sense that should a stereotyper desire to unmount it upon a standard metal base, all that is necessary is to pry the plate loose 95 from the block and the paper will split along its center line displaying a clean, uniform dimension. This obviates the danger of removing or unmounting nailed phenolic plates from wooden blocks, as there is frequently 100 a possibility of breaking off a portion of the brittle printing plate through carelessness or accident. However, when the plate is cemented to the block as just described, it can be quickly removed without any such 105 danger.

While I have herein shown and described certain preferred embodiments of my invention, I wish it to be understood that I do not limit myself to all the details set 110 forth, as modification and variation may be made without departing from the spirit of the invention or exceeding the scope of the appended claims.

What I claim is:

1. A printing plate comprising a printing portion, a backing slab therefor, and a layer of phenolic treated fibrous material and a layer of cement interposed between the printing portion and the backing slab and 120 uniting the two in a manner to prevent the warping or buckling of the printing portion.

2. A printing plate comprising a printing portion, a backing slab therefor, and a layer of fibrous material, and a layer of glue-like cement interposed between the printing portion and the backing slab and uniting the two in a manner to prevent the warping or buckling of the printing portion. 125

3. A printing plate comprising a printing 130

- portion, a backing slab therefor, and a layer of paper and water-glass cement interposed between the printing portion and the backing slab and uniting such portion and slabs.
5. A printing plate comprising a printing portion having phenolic material as a constituent thereof, a fibrous sheet secured to the back of the printing portion, a backing slab for the printing portion, and a suitable cement uniting the backing slab with the fibrous sheet at the back of the printing portion.
10. A printing plate comprising a printing portion including phenolic material, a phenolic treated sheet secured to the back of the printing portion, a backing slab containing phenolic material, and a glue-like cement uniting the backing slab with the phenolic treated sheet at the back of the printing portion.
15. A printing plate comprising a printing portion, a backing slab cemented to the back of the printing portion to prevent the buckling of the latter, said backing slab comprising a fibrous body having a hard and set synthetic resinous material incorporated therein, and a base block fastened to the back of the backing slab.
20. A printing plate comprising a printing portion, a backing therefor comprising a fiber sheet impregnated with a hard and set phenolic material to form the backing slab, and means for cementing the printing portion to the backing slab in a manner to prevent the buckling of the printing portion.
25. The herein described method which comprises applying a fibrous sheet to the back portion of a printing plate, providing a backing slab, and cementing the backing slab to the fibrous sheet under pressure, applying a second fibrous sheet to the back face of the backing slab, and then uniting the parts under pressure.
30. The herein described method which comprises applying a phenolic treated sheet to the back portion of a printing plate, providing a backing slab, cementing the backing slab to the phenolic treated sheet under pressure, applying a second phenolic treated sheet to the back of the backing slab, and then cementing said backing slab to a base block.
35. The herein described method which comprises applying a phenolic treated sheet to the back portion of a printing plate, providing a backing slab, cementing the backing slab to the phenolic treated sheet under pressure, applying a second phenolic treated sheet to the back of the backing slab, and then cementing said backing slab to a base block.
40. Signed at New York city in the county of New York and State of New York, this 5th day of December, A. D. 1919.
45. EMIL E. NOVOTNY.